

# UNITED STATES PATENT OFFICE.

HENRY MATTHEW WELLS, OF ST. ANNES-ON-SEA, NEAR BLACKPOOL, AND JAMES EDWARD SOUTHCOLBE, OF BIRKENHEAD, ENGLAND.

## LUBRICATING-OIL.

1,319,129.

Specification of Letters Patent. Patented Oct. 21, 1919.

No Drawing.

Application filed March 19, 1918. Serial No. 223,378.

To all whom it may concern:

Be it known that we, HENRY MATTHEW WELLS and JAMES EDWARD SOUTHCOLBE, subjects of the King of Great Britain, residing, respectively, at St. Annes-on-Sea, near Blackpool, in the county of Lancaster, and Birkenhead, in the county of Chester, both in the Kingdom of England, have invented certain new and useful Improvements 10 in Lubricating-Oils, of which the following is a specification.

This invention relates to improvements in lubricating oils. It has long been recognized that for many purposes mineral hydrocarbon oils do not lubricate so well as animal or vegetable saponifiable oils and fats and accordingly "compounded lubricating oils" have been largely used, which consist of mixtures of mineral oils with saponifiable 20 oils and fats.

We have discovered that the active principle which enables such saponifiable oils to improve the lubricating properties of mineral oils is a relatively small quantity of 25 free fatty acid, either preexisting in the saponifiable oil, or formed therefrom by hydrolysis during lubrication. Our invention therefore consists primarily in replacing a relatively large amount of saponifiable 30 oil or fat by a relatively minute amount of a suitable free fatty or other organic acid.

It will be seen that the principle underlying our invention is in direct opposition to prevailing views, and it will be desirable 35 therefore to explain the rationale of the process.

Hitherto it has been considered that free fatty acid is a constituent to be rigorously excluded from a lubricating oil, on account 40 of the fear of corrosion. We approached this problem by making a study of the capillary properties of various oils, using the drop pipette to measure the interfacial tension between oil and water. The first result 45 of our work was to show that the saponifiable oils or compounded oils showed a low interfacial tension against water. We next demonstrated that this low interfacial tension was due to the presence of small 50 quantities of free fatty acids, and concluded that the efficacy of the saponifiable oils depended on their free acid content and that in fact these oils merely acted as carriers of free acid.

Accordingly we added free fatty acid

alone to a mineral oil and discovered that the lubricating properties were greatly improved while the interfacial tension against water was correspondingly lowered.

Our invention presents three great advantages over existing practice:—

(1) By isolating the "active principle" we are enabled to produce oils of widely varying properties as will be described hereafter.

(2) We are enabled to replace a large amount of saponifiable oil or fats in a compounded lubricant by a small amount of free fatty or organic acid and thus obtain a better product at a much less cost. The saving in saponifiable oil is especially important since we can prepare valuable products while liberating large quantities of saponifiable oils for use as foods.

(3) In actual practice we find that far 75 from increasing the danger of corrosion we are enabled to minimize it.

In our products the amount of fatty acid is small and limited; whereas in the usual commercial products, the amount may be 80 small initially but it is potentially very large. Owing to hydrolysis during lubrication the percentage of fatty acid in a compounded oil containing say ten per cent. of saponifiable oil is potentially equal to a 85 very large fraction of this ten per cent. The danger from corrosion is large and uncontrollable. It is this factor which made it impossible to avoid corrosion completely by employing lubricating oils containing (initially) the minimum quantity of free fatty acid. Our experiments show that on the contrary a small quantity of free fatty acid is 90 essential but that the free fatty acid should be added as such, so that its amount is limited and cannot increase, whereas if the free acid is present as the impurity or hydrolytic product of a saponifiable oil, its amount can 95 increase very largely.

The free acid, preferably free fatty acid, 100 e. g., commercial olein containing 95% free acid, and / or whale oil fatty acids either hardened or not may be added in quantities of 1 to 2% to the mineral oil, or the free fatty acid may be incorporated with a small 105 quantity of mineral oil, and this active mixture may be diluted with mineral oil as required. Many of the advantages of the invention may be obtained by incorporating the free fatty acid with a small quantity of 110

2 saponifiable oil as vehicle but it is desirable to employ mineral oil for this purpose.

The choice of the free acid is dependent on the lubricating and other properties desired. Broadly speaking, the best free organic acid to use is that which is obtained from the fatty oil whose properties it is desirable to reproduce. Thus rape oil and cocoanut oil impart different properties to the compounded oils made therefrom and these properties may also be imparted by adding small quantities of the free fatty acids corresponding thereto.

In theory the process depends on the principle that lubrication is a function of the capillary properties of the oil. A satisfactory lubricant must "wet" the bearing surfaces so that a thin film of lubricant will tend to move into the constricted areas of great pressure. Now in practice the bearing surfaces are usually contaminated with a film of moisture and there is a liability to form oxid films. The action of the free acid is to lower the interfacial tension between oil and water and the mechanism of the process is apparently to allow the oil to displace the water film from the bearing surface. The chemical affinity between the acid and the metallic surface or the oxid film (if present) runs parallel with a similar reduction in interfacial tension which has similar results.

The action of the free fatty or other acid depends on its molecular weight. If any acid of very low molecular weight such as butyric acid is used it will exert a deemulsifying effect and we can therefore apply our process to produce non-emulsifiable mineral oils. This is of great importance in certain classes of work where the oil is violently agitated with water and much trouble is experienced through emulsification. On account of the low molecular weight, these acids are much more active and it is not desirable to exceed the limit of 1%.

On the contrary certain fatty acids of high molecular weight possess the property of increasing the emulsibility of hydrocarbon oils which is of importance in certain cases of lubrication. Thus certain highly unsaturated acids of high molecular weight are especially active. This is probably associated with the phenomena of polymerization and soap formation.

55 Our invention is thus based on adding to a mineral oil a relatively minute amount of a compound which lowers the interfacial tension between the oil and water in the manner described.

60 Any hydrocarbon oil may be used, *e. g.*, from petroleum, coal tar, shale, colophony, etc.

65 Fatty acids are very suitable additions; the commercial products are satisfactory. They may be obtained from any class of

saponifiable oil fat soap or recovered grease. We may also use the so-called naphthenic acids or other acids obtained or manufactured from raw petroleum, shale, coal-tar or colophony.

70 The invention may be applied to improve the lubricating properties also the emulsifying and / or the deemulsifying properties of mineral oils.

We shall now give examples showing the 75 application of our invention but it will be understood that these are merely illustrative.

#### *Example I.*

2 % of commercial olein (fatty acid) or 80 the like is incorporated with a good quality mineral lubricating oil. A product is obtained resembling closely a compounded oil containing 10 to 20% of olive oil, lard oil or tallow.

#### *Example II.*

A concentrated compound is prepared containing equal weights of commercial fatty acids and mineral oil by warming and mixing these ingredients. This concentrated compound is added to a hydrocarbon oil to the extent of 3% by weight (=1% fatty acid).

#### *Example III.*

95 A non-emulsifying oil is prepared by adding 0.8% of butyric, cinnamic or an oil-soluble sulfonic acid to hydrocarbon oil. Certain naphthenic acids also exert this demulsifying effect.

#### *Example IV.*

An emulsifying oil suitable for marine lubrication or the like is produced by adding 1% of the acids obtained from rape oil or 105 wool-grease and the like to a viscous hydrocarbon oil.

The product closely resembles a compounded oil made from hydrocarbon oil and blown rape oil.

#### *Example V.*

110 A mineral oil of high viscosity is treated with 2% of the commercial acids from castor oil or even with 2% of olein. The product is similar in properties to castor oil at relatively not too high temperatures, and is very suitable for lubrication of aeroplane engines.

115 We declare that what we claim is:

1. A lubricating oil consisting of a hydrocarbon oil containing a relatively minute amount of a substance which lowers the surface tension of said oil against water without admixture of more than a correspondingly minute amount of saponifiable glycerid.

120 2. A lubricating oil consisting of a hydrocarbon oil containing a relatively minute amount of a free organic acid, without more 125

130

- than a substantially equal amount of saponifiable glycerid.
3. A lubricating oil consisting of a hydrocarbon oil containing a relatively minute amount of a free fatty acid unaccompanied by more than a correspondingly minute amount of saponifiable glycerid.
4. A lubricating oil consisting of a hydrocarbon oil containing about one to two per cent. of free fatty acids.
5. A lubricating oil to replace a compound lubricating oil consisting of a hydrocarbon oil plus a relatively large amount of a saponifiable glycerid, characterized by the replacement of said glycerid by a relatively minute amount of the corresponding fatty acid derived from said glycerid.
6. A lubricating oil consisting of a mineral oil highly viscous at atmospheric temperatures, containing a small quantity of commercial fatty acid substantially without
- addition of more than a correspondingly relatively small amount of castor oil.
7. The process of preparing a compound lubricating oil from hydrocarbon oil, which consists in admixing a free fatty acid with a substantially equal amount of hydrocarbon oil and adding a predetermined amount of said mixture to the oil to be compounded.
8. A hydrocarbon oil containing a viscous mineral oil and approximately two per cent. of fatty acids derived from castor oil.
- In witness whereof, we have hereunto signed our names this 1st day of March, 1918, in the presence of two subscribing witnesses.

HENRY MATTHEW WELLS,  
JAMES EDWARD SOUTHCOMBE.

Witnesses:

HAROLD EDWIN POTTS,  
RICHARD WHIMSTER ELAND.